

April 14, 1925.

1,533,606

R. P. PERRY

PROCESS OF PRODUCING RECEPTACLES

Filed Dec. 16, 1920



*Fig. 1.*



*Fig. 2.*



*Fig. 3.*

INVENTOR

*Ray P. Perry*

BY

*Chas. W. Mattner*

ATTORNEY

Patented Apr. 14, 1925.

1,533,606

# UNITED STATES PATENT OFFICE.

RAY P. PERRY, OF UPPER MONTCLAIR, NEW JERSEY.

## PROCESS OF PRODUCING RECEPTACLES.

Application filed December 16, 1920. Serial No. 431,099.

*To all whom it may concern:*

Be it known that I, RAY P. PERRY, a citizen of the United States, residing at Upper Montclair, in the county of Essex and State of New Jersey, have invented certain new and useful Improvements in Processes of Producing Receptacles, of which the following is a specification.

This invention relates to a process for forming receptacles from sheets containing fibrous material and waterproofing material, and to the product thereby formed.

One of the objects of this invention is to provide a receptacle of this character that shall be impervious to water, shall be capable of withstanding mechanical stress or strain, shall possess good wearing qualities, and shall present a pleasing appearance. Another object is to produce a receptacle in which the fibers are somewhat aligned and the bottom and sides of the receptacle are firmly united into a substantially integral and homogeneous article.

In practicing this invention I prepare a sheet of material in an ordinary paper-making machine, which sheet contains fibrous material, such as paper-making stock, and waterproofing material. This sheet is wrapped or wound around a former to constitute the sides of the receptacle, and disks are cut from the sheet to form the bottom of the same. The sides and bottom of the receptacle are firmly united by the application of the proper amount of heat and pressure.

The invention will be understood from the description in connection with the drawings, in which

Fig. 1 is a side elevation indicating something diagrammatically apparatus for forming the sheet.

Fig. 2 is a side view partly in section showing a press for the receptacle.

Fig. 3 is a side view partly in section showing a modified form of the press.

In the drawings reference character 1 indicates the vat of an ordinary paper-making machine in which there is a foraminous cylinder 2, upon which the sheet 3 is formed in the usual way. A batch of fibrous paper stock and comminuted waterproofing material is introduced into the vat 1, and a sheet 3 is formed therefrom on the cylinder 2 and picked up by means of the wet blanket 4, which passes over rolls 5 and 6. The sheet 3 may be passed between the rolls 6

and 7 to remove a portion of the water, after which it is rolled upon a former 8 into a number of convolutions 9 sufficient to form the sides of the receptacle, whereupon the sheet 3 is severed. The sheet is preferably wound up in a wet condition, whereupon the fibers along adjacent surfaces will felt or mat to produce an initial joining of the successive convolutions.

A number of disks 10 having diameters equal to the outside diameter of the convolutions 9 are cut from the sheet 3 and superposed upon each other to provide a disk of sufficient thickness to constitute the bottom of the receptacle.

The plurality of disks 10 are placed in the bottom of a circular opening 11 in the base 12 of a press, and the roll of convolutions 9 is placed upon the disks 10 with the end 9' of the convolutions in contact with the circumferential edge of the top one of the disks 10. If necessary, a small amount or thin layer of bituminous material may be applied between the disks 10 and the end 9'. The convolutions 9 fit closely within the opening 11, and the metal cylinder 13 fits closely the inside of the convolutions 9.

A pressure member 14 operated by the plunger 15 fits around the cylinder 13 and is capable of passing inside of the opening 11 of the base 12. The base 12 is provided with a heating chamber 16 into which heating and cooling fluids may be introduced and withdrawn through the pipes 17 and 18, and the cylinder 13 is similarly provided with a heating chamber 19 into which heating and cooling fluids may be introduced and withdrawn through the pipes 20 and 21. A plunger 15 carries an adjustable plate 22 which contacts with the upper end of the cylinder 13 to apply pressure thereto at the proper time.

The operation of the press shown in Fig. 2 is as follows:

The receptacle, consisting of the plurality of disks 10 and the convolutions 9, is inserted in the opening 11, and the cylinder 13 is inserted inside the convolutions 9. The receptacle is heated sufficiently to melt the waterproofing material by introducing heating fluid into the heating chambers 16 and 19. The pressure member 14 is then caused to descend and compress the convolutions 9 in a vertical direction or longitudinally of the axis of the receptacle. The plunger 15 slides in the space between the cylinder 13

and opening 11, and when the convolutions 9 have been compressed approximately to the desired extent, the plate 22 contacts with the upper end of the cylinder 13, thereby applying pressure to said cylinder and causing the same to compress the disks 10 to the desired extent. The melted bituminous material spreads uniformly, and the convolutions and disks are firmly united into a substantially integral and homogeneous product. The heating fluid is withdrawn from the chambers 16 and 19 and cooling fluid is introduced therein, whereupon the waterproofing material is caused to "set", thus causing the receptacle to become rigid and retain its shape. The pressure member 14 and the cylinder 13 can be withdrawn, after which the integral receptacle can be taken out of the opening 11.

20 In the modification shown in Fig. 3 the opening 11' of the base 12' is made in the shape of an inverted truncated cone and the pressure member 14' is correspondingly shaped. The base 12' is provided with a heating and cooling chamber 16', and the pressure member 14' is provided with a heating chamber 19' similar to those mentioned in connection with Fig. 2.

30 In practicing the process using the press shown in Fig. 3, the convolutions 9<sub>3</sub> will be formed in the shape of a cylinder, one of whose ends has a smaller diameter than the other, in any convenient manner, as for example by winding the sheet 3 upon a mandrel having the shape of a tapered cylinder. The disks 10' to form the bottom of the receptacle and the convolutions 9<sub>3</sub> to form the sides thereof are placed in the opening 11', and after being heated sufficiently to 40 melt the waterproofing material the pressure member 14' is caused to descend and apply the proper amount of pressure. In this press the descent of the pressure member 14' will cause the material constituting the convolutions to be pressed outwardly in a somewhat radial direction instead of causing the same to be compressed longitudinally, as indicated in Fig. 2. The parts will be so proportioned that the bottom end 45 of the pressure member 14' will come into contact with and compress the bottom disks 10' at the moment when sufficient densification of the convolutions 9<sub>3</sub> has taken place. It is obvious that by having the opening 11' 50 of sufficiently small diameter to prevent the convolutions 9<sub>3</sub> from reaching the bottom of the opening 11' before pressure is applied, the convolutions can be made to slide downwardly so that there is substantially 55 the same decrease in the outside diameter of the convolutions 9<sub>3</sub> as there is increase in the inside diameter of the same, while the pressure or densification is caused to take place, thus rendering it less likely that any 60 of the fibers will be torn apart or greatly 65

displaced from the positions in which they were matted or felted together on the former indicated in Fig. 1.

It will be seen that since the fibers in the sheet 3, by means of a paper-making machine, will lie very largely in directions longitudinally of the sheet, the receptacle will be such that when the pressure is applied, either as indicated in Fig. 2 or as indicated in Fig. 3, it will be perpendicular to the sides of the fibers, and the fibers as a whole will not be compressed in a direction longitudinally of the length of the fibers themselves. Also, the receptacle when completed will have the fibers in the sides thereof lying in circumferential paths and those in the bottom thereof lying parallel to the bottom, so that moisture is less likely to penetrate the receptacle, as the fibers are not parallel to the path that the moisture 85 would take in passing through the bottom or sides of the receptacle.

Instead of uniting the bottom to the convolutions, as above described, the convolutions themselves may be compressed to densify and unite the same, thus forming a rigid conduit in which the fibers are nearly all lying in circumferential lines.

Instead of making the convolutions circular and making the bottom of the receptacle in the shape of disks, I may make the convolutions of other shapes, such as square or rectilinear, etc., and the cut-out portions of the sheet to form the bottom of the receptacle will be correspondingly shaped.

Pitch has been found to be a very convenient and suitable material to use as the waterproofing material, and pitch of a melting point of about 250° F. to 300° F. to give a very rigid and strong product, when the pitch is used in sufficient quantities so that the final product consists of from about 50% to 90% by weight of pitch. The application of the heat and pressure may reduce the volume of the mixed fibrous and waterproofing material about one-half its original volume, so that the density of the final product may be approximately the same as that of the waterproofing material itself.

In using the term "receptacle" I do not intend to be restricted to a vessel having a closed end, but intend to include conduits and the like and the term is to be so understood in the specification and claims.

I claim:

1. The process which comprises forming a receptacle from a sheet containing felted fibrous material and waterproofing material in which a large percentage of said fibers extend in the same general direction, and pressing said receptacle in directions substantially perpendicular to said fibers and substantially parallel to the axis of said receptacle.

2. The process which comprises forming

- a receptacle from a sheet containing felted fibrous material and comminuted waterproofing material in which a large percentage of said fibers extend in the same general direction, and pressing said receptacle in directions substantially perpendicular to said fibers at such a temperature that said waterproofing material is melted.
3. The process which comprises forming a receptacle from a sheet containing felted fibrous material and waterproofing material in which a large percentage of said fibers extend in the same general direction, pressing said receptacle in directions substantially perpendicular to said fibers at such a temperature that said waterproofing material is melted and at such a pressure that the density of the receptacle becomes substantially the same as that of said waterproofing material.
4. The process which comprises forming a sheet containing felted fibrous material and waterproofing material so that the fibers lie in one general direction, forming a receptacle from a plurality of layers of said sheet and hot pressing the same in an axial direction.
5. The process which comprises forming a sheet containing felted fibrous material and waterproofing material so that the fibers lie in one general direction, forming a receptacle from a plurality of layers of said sheet and hot pressing the same in a direction perpendicular to said fibers.
6. The process which comprises forming a receptacle from a sheet containing felted fibrous material and pitch in which a large percentage of said fibers extend in the same general direction, and pressing said receptacle in directions substantially perpendicular to said fibers.
7. A receptacle closed at one end, the sides of which are made of a plurality of layers of mixed fibrous and bituminous materials which have been united by heat and pressure.
8. A receptacle closed at one end, the sides of which are made of a plurality of layers of mixed fibrous and bituminous materials which have been united by heat and by pressure applied in an axial direction, said fibers lying generally in circumferential directions.
9. A receptacle closed at one end, the sides of which are made of a plurality of layers of mixed fibrous and bituminous materials which have been united by heat and by pressure applied in an axial direction, said fibers lying mainly in planes at right angles to the axis of said receptacle.
10. A receptacle closed at one end, the sides of which are made of a plurality of sheets of mixed fibrous material and comminuted pitch which have been united by heat and by pressure applied in a substantially axial direction.

In testimony whereof I affix my signature.  
RAY P. PERRY.